

## UNITED STATES PATENT OFFICE

2,282,703

## ASPHALT PREPARATION

Robert E. Burk, Cleveland, Ohio, assignor to The Standard Oil Company, Cleveland, Ohio, a corporation of Ohio

No Drawing. Application October 28, 1936,  
Serial No. 108,052

8 Claims. (Cl. 106—269)

This invention relates to asphalt preparation; and it is among the objects of the invention to provide a product having durability and resistance to change of properties in service. Other objects and advantages will appear as the description proceeds.

To the accomplishment of the foregoing and related ends, the invention, then, comprises the features hereinafter fully described, and particularly pointed out in the claims, the following description setting forth in detail certain illustrative embodiments of the invention, these being indicative however, of but a few of the various ways in which the principle of the invention may be employed.

The invention will be best understood by reference to an illustrative example:

A petroleum residuum, as a pipe still bottoms of Mid-Continent petroleum left after the various cuts have been taken off through lubricating fractions, and having for instance a flash point of 550° F., and penetration of about 200 at 77° F., is subjected to oxidation by blowing with air, and maintaining an effective temperature of 400-550° F., samples being taken until the material shows desired characteristics, as for example 12 to 25 penetration at 77° F., and melting point 150-235° F., the oxidizing process requiring many hours, for instance 2 to 24 hours, depending somewhat upon the constancy of maintenance of action. With the oxidized material there is finally incorporated, while it is in sufficiently fluent condition, 0.1 per cent of a naphthenate of a heavy metal, as cobalt, manganese, iron, lead, vanadium, or zinc, being thoroughly disseminated.

While the naphthenic salts are particularly desirable, I may in some instances employ salts of oleic, linoleic, tung acids, and synthetic carboxylic acids made by oxidizing petroleum, with metals as aforesaid.

In general, the amount of the naphthenic or other salt is small, for instance 0.001-1 per cent. The agent, it is noted also, is to be added after active reaction has passed in the asphalt, or at least if added before there must be sufficient to insure the finished product containing an amount of the metal compound as indicated.

I have found further that the action of the salts of the heavy metals as aforesaid, is promotive with respect to each other, and a mixture thereof yields results out of proportion to and much greater than the total of the respective individuals entering into the mixture. Thus, such mixtures as cobalt naphthenate and man-

ganese linoleate or tungate, or the lead salts of synthetic carboxylic acids made by oxidizing petroleum, as now commercially available, may be employed with zinc oleate or linoleate. And, variously, mixtures of the salts may be employed as desired.

If the agent is added before oxidation is complete, I have found further that the heavy metal in the form of reactive hydroxide or oxide or hydrous oxide may advantageously be employed instead of or in addition to the pre-formed salt of the metal. Incorporation thus of amounts of cobalt hydroxide, zinc oxide, litharge and like compounds of the said heavy metals reactive with carboxylic acids are desirable, reaction by the oxidation acids formed by the action of the oxygen in the blowing process on the petroleum hydrocarbons yielding corresponding amounts of salts of the metals to become effective as if added pre-formed.

Asphalts in accordance with the invention show a particularly good surface after application to point of usage, as in exposure on roofing, walls, and other surfaces, the customary tendency heretofore of asphalt to develop surface cracks, and also generally rapidly accumulate a coating of dust and dirt, being absent.

Other modes of applying the principle of the invention may be employed, change being made as regards the details described, provided the features stated in any of the following claims, or the equivalent of such, be employed.

I therefore particularly point out and distinctly claim as my invention:

1. A process of making asphalt, which consists in oxidizing petroleum residuum by heating and agitating in exposure to oxygen and thickening the material to desired melting point and penetration, and after such oxidizing incorporating a small amount of a naphthenate of a metal of the group consisting of cobalt, manganese, iron, lead, vanadium and zinc.

2. A process of making asphalt, which consists in heating and agitating petroleum residuum in exposure to oxygen and thickening the material to desired melting point and penetration, and after such oxidizing incorporating a small amount of a salt of a carboxylic acid of the group consisting of naphthenic, oleic, linoleic, tung acids and oxidized petroleum acids, with a metal of the group consisting of cobalt, manganese, iron, lead, vanadium and zinc.

3. A process of making asphalt, consisting in oxidizing petroleum residuum by heating in exposure to oxygen and thickening the material to

desired melting point and penetration, and after such oxidation incorporating a small amount of mixed salts of acids of the group consisting of naphthenic, oleic, linoleic, tung acids and oxidized petroleum acids, with metals of the group consisting of cobalt, manganese, iron, lead, vanadium and zinc.

4. A process of making asphalt, consisting in oxidizing a petroleum residuum by heating in exposure to oxygen and thickening the material, and then incorporating a small amount of a compound of a metal of the group consisting of cobalt, manganese, iron, lead, vanadium and zinc.

5. A process of making asphalt, consisting in oxidizing petroleum residuum by heating in exposure to oxygen and thickening the material, and then incorporating a small amount of a reactive compound of the group consisting of oxides, hydroxides, and hydrous oxides of metals

of the group consisting of cobalt, manganese, iron, lead, vanadium and zinc.

6. Asphalt, consisting of oxidized asphalt and a small amount of a naphthenate of a metal of the group consisting of cobalt, manganese, iron, lead, vanadium and zinc.

7. Asphalt, consisting of oxidized asphalt and a small amount of a salt of an acid of the group consisting of naphthenic, oleic, linoleic and tung acids with a metal of the group consisting of cobalt, manganese, iron, lead, vanadium and zinc.

10 8. Asphalt, consisting of oxidized asphalt and a small amount of a mixture of salts and acids of the group consisting of naphthenic, oleic, linoleic, tung acids and oxidized petroleum acids, with a metal of the group consisting of cobalt, manganese, iron, lead, vanadium and zinc.

15 ROBERT E. BURK.